

Oct. 17, 1939.

M. J. UDY

2,176,686

CHROMIUM ALLOY STEEL MANUFACTURE

Filed Jan. 22, 1938



INVENTOR

MARVIN J. UDY

BY

Pennie, Davis, Marvin & Edmonds  
ATTORNEYS

Patented Oct. 17, 1939

2,176,686

# UNITED STATES PATENT OFFICE

2,176,686

## CHROMIUM ALLOY STEEL MANUFACTURE

Marvin J. Udy, Niagara Falls, N. Y.

Application January 22, 1938, Serial No. 186,465

18 Claims. (Cl. 75—27)

This invention or discovery relates to chromium alloy steel manufacture; and it comprises as a new article of manufacture useful in making low carbon chromium-iron alloys a solid mass, advantageously in the form of briquettes, or blocks, capable of undergoing internal reactions with production of a molten body of such an alloy, said mass being composed of an intimate admixture of a finely ground iron oxide, fine 5 grained ferrochrome silicon low in carbon, high in silicon and in proportion to reduce the iron oxide and finely divided lime in amount to convert the silica to be formed in the reduction into a basic lime silicate slag; and it further comprises 10 processes of utilizing chromite ores for making low-carbon chromium-iron and chromium-steel alloys wherein a ferrous chromite ore of any grade is reduced with carbon to high carbon ferrochromium with elimination of the ore gangue, 15 the ferrochromium is re-smelted with silica and carbon to a highly siliconized ferrochrome metal low in carbon and this metal, carrying most of the chromium and iron of the original ore, is mixed in finely divided form with iron oxide and lime, and the silicon of the metal is removed 20 therefrom and replaced with iron by exothermic reduction of the iron oxide forming the low carbon chromium-iron alloy and a basic slag, both in molten form and readily separable; all as more 25 fully hereinafter set forth and as claimed.

In nearly all the commercial chromium-iron alloys such as stainless steel, rustless iron, etc., a low carbon content is required. The chromium content may vary from a fraction of one per cent 30 up to 30 per cent or over. Other alloying metals are usually present. In nearly all cases these alloys have been produced by the use of commercial ferrochromium having chromium in a ratio to iron of around 70:30. The reason for 35 using these high chromium ferro alloys is that they are correspondingly low in the ratio of carbon to chromium. They can be produced only from the highest grade chromite ores low in iron content. It is an economic waste to use high 40 grade ores to produce a rich ferrochromium and then dilute this metal with more iron to form commercial alloys in which chromium is only a minor constituent.

It is an object achieved in the present invention to provide a material and method for 45 making the low carbon finished steel or iron alloyed with chromium and other metals in minor proportions without dependence upon high grade chromite ores of low iron ratios. It is no longer 50 necessary to "high grade" the natural chromite

ore deposits of the world and to leave unutilized plentiful supplies of rich ferrous chromite mineral because of its low chromium to iron ratio.

I have discovered that iron-chromium alloys of predetermined chromium and carbon contents are made with great facility by exothermic reaction, in finely divided admixture, of iron oxide with ferrochromium siliconized to low carbon and high silicon contents sufficient to reduce the iron oxide and with an amount of lime to convert 10 the silica formed in the reduction to a silicate slag containing lime in more than an equimolecular ratio to the silica. The iron oxide in being reduced to iron by silicon dilutes the chromium and the reaction heat of the finely 15 divided admixture is in excess of the amount required to melt the silicate; both the dilution and the excess heat, as well as the carbon content of the metal product, being predetermined by the percentage of silicon in the ferrochrome-silicon, 20 that is by the degree of siliconization of the ferrochromium in admixture with iron oxide. As I have found, the silicon in the ferrochrome-silicon component with admixed lime in more than a 2:1 proportion by weight to the silicon 25 protects the chromium against oxidation by the iron without requiring silicon in great excess. The lime in the mixture combining with silica promotes the oxidation of silicon by iron oxide and adds to the heat of the internal reaction 30 taking place in the mixture when ignited.

A silico-thermic briquetted mixture of ferrochrome silicon, iron oxide and lime, in proportions giving on reaction a basic silicate slag and a chromium-iron metal containing residual 35 silicon in amounts of the order of 1 per cent of the metal or less and a low carbon content resulting from dilution of the low-carbon ferrochrome metal by the exothermically reduced iron, is a highly advantageous material for making any oxidation-resistant high strength alloy 40 steel or iron. One of its outstanding advantages is that it can be made from chrome iron ores of any chromium-iron ratio, even from an iron ore containing minor amounts of chromium, for example, a Cuban iron ore of 2-4 per cent chromium content or a 1:20 chromium-iron ratio. Another advantage is that there can be incorporated in the silico-thermic mixture other alloying constituents such as nickel, molybdenum, 45 manganese, vanadium, tungsten, etc. wanted in the finished metal. These may be incorporated either as oxides in the iron oxide component or as metals in the ferrochrome silicon component. In the latter case silicate ores of the metals can be 50 55

utilized as sources of silicon for the siliconized metal. These other alloying metals may, however, be added to the molten chromium-iron metal formed upon ignition of the mixture and exothermic reaction therein. The metal product of reaction of the three-component mixture may be diluted further with molten steel or iron to adjust the chromium content as desired.

It is sometimes advantageous to incorporate in the mixture some saline oxidant as sodium chlorate, or nitrate or chromate, with excess ferrochrome silicon over that needed to reduce the iron oxide. This gives heat in oxidizing silicon without diluting the ferrochrome metal with iron. It increases the amount of heat available for melting the slag and the metal. The exothermicity of the mixture may thus be increased. It is usually better to have the proportion of iron oxide and saline oxidant to the silicon a little less than that sufficient to oxidize all the silicon. A little silicon in the metal in the presence of lime protects the chromium from oxidation. Chromate used as oxidant adds chromium to the metal.

I have found it highly advantageous to add to the exothermic mixture a small proportion of chromated ferrichromite made by roasting high carbon chromium or ferrochromium.

Not the least of the advantages of the silico-thermic material for making alloy steel is that it can be directly converted into such an alloy by being introduced into an open hearth steel furnace hot enough to start the exothermic reaction within the material. An ordinary steel making temperature around 1500 to 1600° C. is advantageous and the material, which may carry within itself all or the greater part of the heat energy required to melt the reaction products to a free running metal and slag, may be slowly fed to the furnace. Thus working, any deficiency of heat required to finish the alloy, or to add metallic alloying constituents in addition to the chromium, may be supplied by the usual means for heating the furnace. This allows some latitude in the silicon content of the siliconized ferrochromium, which in the last analysis determines the amount of heat delivered by the reaction mixture per unit weight of the material.

The amount of heat developed, and therefore the temperature, depends on the amount of silicon plus iron oxide in the silico-thermic mixture and where foreign heat can be utilized, as in working in a hot furnace, it is possible to diminish somewhat their proportion and increase concomitantly the proportion of other useful constituents.

High carbon ferrochromium made from chromite ore of any grade by well known smelting methods is readily siliconized to any desired extent up to, say, 75 percent by smelting with silica and carbon as coke. Ferrochrome-silicon thus made and containing 50 per cent silicon or more is extremely low in carbon content. This metal in admixture with iron oxide and lime, in proportions as described, is converted by exothermic action in an open hearth steel furnace to a carbon-free metal of a diluted chromium content and a lime silicate slag; with development of a quantity of heat not far from that needed to melt the diluted metal and the slag. In the reaction,  $3\text{Si} + 2\text{Fe}_2\text{O}_3 = 4\text{Fe} + 3\text{SiO}_2 + 223,600$  calories, each unit of silicon in ferrochrome-silicon being replaced by 2.66 units of iron, a 70:30 ferrochrome with 50 per cent Si, for example, is diluted to 18 75 per cent chromium metal, or 3.66 pounds per

pound of silicon; the silicon being converted with lime into 4.5 to 5 pounds lime silicate slag. A positive heat development in the silicate formation of 900 cal. per unit Si, added to 2600 cal. for the reduction brings the exothermic heat to 3500 centigrade units per pound Si. This amount of heat balances 1500 heat units used in melting 3.68 pounds metal and 2000 units in 4.5 to 5 pounds slag. The production of carbon-free 18 per cent chromium metal from a mixture of 10 ferrochrome silicon and iron oxide with a slag ratio of 1.25 may thus be made self sustaining.

In some cases it may be advantageous to siliconize the ferrochrome component to a moderate silicon content of 30 to 40 per cent in order to 15 increase the proportion of chromium or other alloying metal in the silicon-thermic material. This may avoid undue dilution of the chromium by iron in the finished alloy. But it is usually better to run the silicon up to 50 per cent or more 20 of the ferrochrome silicon so as to have more latent available heat to add to the heat of the steel furnace. By adding sodium chlorate or chromate or nitrate silicon supplies heat without diluting the metal with iron formed in reduction of iron oxide.

It may be noted that the higher the percentage of silicon in the ferrochrome silicon, the lower is the carbon content and the greater is the dilution of the ferrochrome and the carbon content 30: with iron replacing the silicon by virtue of the reduction of the oxide component in the silico-thermic mixture. Thus high silicon in the ferrochrome component conduces in two ways to low carbon in the alloy steel made by igniting the 35: mixture.

As to the silicon content of the ferrochrome silicon, it is found that a given silicon content insures a lower carbon content, the lower the ratio of chromium to iron in the ferrochromium 40 which is siliconized. For example, in a ferrochromium of a Cr-Fe ratio 1:1 or less, 40 per cent Si insures a carbon content under 0.1 per cent. With extremely low chromium contents, under 5 per cent, carbon is below 0.10 per cent with 10 45 to 20 per cent Si in the metal. Thus there is particular advantage in utilizing substandard chromite ores for making the ferrochromium to be siliconized. For example, a 40 per cent silicon metal of a 1:1 Cr/Fe ratio can be converted to 50 an 18 per cent chrome steel of a carbon content under 0.10 per cent by exothermic reaction with lime, iron oxide and sodium chlorate or nitrate in proportions giving a reaction heat sufficient to melt the metal and silicate slag. If a somewhat larger chromium content in the steel is required, it may be obtained by putting a somewhat smaller silicon content in the ferrochrome silicon to be replaced by iron. If a smaller chromium content is wanted in the chrome steel, it 60 is a simple matter to dilute with iron the chrome-iron alloy formed by reaction of the silico-thermic mixture. Likewise, the chromium content of the finished alloy is raised or lowered by incorporating more or less saline oxidant in the silico-65 thermic material.

It is advantageous, as I have found, to produce the ferrochrome silicon by siliconizing high carbon ferrochromium made by smelting a chromite ore with carbon in a well known way. In this 70 smelting the process described in my copending application Serial No. 165,954, filed September 27, 1937, (continued in Serial No. 228,861, filed Sept. 7, 1938) gives a high yield of chromium from the ore by putting a small amount of silicon into the 75

metal. This metal can then be smelted with silica and carbon to produce siliconized ferrochromium of a high silicon content which ensures a carbon content of less than 0.1 per cent. As above stated, the low grade or high iron ferrochromiums lend themselves particularly well to lowering the carbon content by addition of silicon. In this operation it may be advantageous to use as source of silicon a nickel silicate ore in order to put into the siliconized metal a desired content of nickel with the chromium. A silicon content of 50 per cent or over is advantageous not only in lowering the carbon content, but also in providing in the silico-thermic mixture a good supply of latent exothermic heat per unit weight of the material.

For the iron oxide to be mixed with the siliconized ferrochromium, mill scale or the magnetic oxide may serve. This requires less heat for reduction per unit of iron than the ferric oxide. But the magnetic oxide dilutes the ferrochrome metal to a greater extent than ferric oxide or hematite. Either of the oxides is available for my purposes; the purer the oxide the better. Oxide ores containing small amounts of oxides of metals desired as minor alloying constituents of the chrome steel alloy may be used to advantage; for example, iron ores containing vanadium oxides.

In a specific embodiment of the invention I use as source of chromium in the exothermic mixture a low grade chromite ore of the following composition:

|                                | Per cent |
|--------------------------------|----------|
| Cr <sub>2</sub> O <sub>3</sub> | 13.85    |
| Iron oxides as FeO             | 12.00    |
| MgO                            | 21.18    |
| SiO <sub>2</sub>               | 35.70    |
| Al <sub>2</sub> O <sub>3</sub> | 2.02     |
| CO <sub>2</sub>                | 14.30    |
|                                | 99.05    |

This ore is reduced in a submerged arc electric furnace with carbon in the presence of lime and silica in proportions giving a normal dibasic silicate slag and an excess of silica for reduction, as described in my mentioned copending application Serial No. 165,954. The reduction results in a high yield of metal having the following composition:

|    | Per cent |
|----|----------|
| Cr | 42       |
| Fe | 48       |
| C  | 7        |
| Si | 3        |

This metal is siliconized by smelting with quartzite and coke to a silicon content of 40 per cent and a carbon content well under 0.10 per cent.

The final reactive mixture for making the finished alloy steel is made up by grinding the ferrochrome silicon to 100 mesh and mixing it with finely ground iron ore containing 60 per cent iron, a small amount of pure nickel oxide, lime and a little sodium chloride as an oxidant for the silicon. The proportions are:

|                                     | Parts |
|-------------------------------------|-------|
| Ferrochrome silicon, 40 per cent Si | 150   |
| Iron ore, 60 per cent Fe            | 210   |
| Nickel oxide (NiO)                  | 23.9  |
| Lime, CaO                           | 192   |
| NaClO <sub>3</sub>                  | 21.2  |

These materials are all ground together in a ball

mill to pass 100 mesh. This mixture is then briquetted, or it can be packed in cans. For ignition of the mixture a temperature of 800° to 900° C. suffices. To make the alloy metal the briquetted mixture is fed to an open hearth furnace heated to 1500° C. The reaction proceeds smoothly and rapidly and there is produced 225 pounds molten steel analyzing as follows:

|          | Per cent |
|----------|----------|
| Chromium | 17.3     |
| Nickel   | 8.3      |
| Carbon   | 0.05     |
| Silicon  | 0.4      |

The slag amounts to 320 pounds, which is in a ratio to the steel of 1.4 to 1.

It is noted that in the above example the saline oxidant sodium chloride is used to leave only a little excess silicon over that required in being replaced by iron to dilute the metal to the desired composition. This is advantageous in increasing the exothermicity of the mixture and it may be utilized to give a fully self-sustaining reaction. It is further noted that by lowering the silicon in the ferrochromium to 35 per cent the reaction with iron oxide gives the same metal composition without the use of chlorate. With the lowered silicon, the slag volume would be less. It is noted that the silicon is used entirely to reduce oxides other than chromium oxide.

In another specific embodiment of my invention I utilize a Puerto Rican limonite iron ore which on roasting analyzes as follows:

|                                                  | Per cent |
|--------------------------------------------------|----------|
| Fe <sub>2</sub> O <sub>3</sub> , Fe 49 per cent  | 70       |
| Al <sub>2</sub> O <sub>3</sub>                   | 23.0     |
| SiO <sub>2</sub>                                 | 2.7      |
| NiO, Ni 0.78 per cent                            | 1.0      |
| Cr <sub>2</sub> O <sub>3</sub> , Cr 1.3 per cent | 1.9      |

I smelt this roasted ore in an electric furnace with coke as reducing agent, producing from 100 parts of ore (according to the process of application Serial No. 165,954), 51 parts of metal containing 49 parts iron, .7 part nickel and 1.2 part chromium. The metal contains about 4 per cent carbon and 4 per cent silicon.

I next smelt this metal with silica and coke to produce 76 parts of a siliconized metal containing 1.58 per cent chromium and 0.92 per cent nickel with 30 per cent silicon and carbon under 0.10 per cent. This melting is readily done in an electric furnace of the submerged arc type. The same smelting can be accomplished in a blast furnace.

The 76 parts of siliconized metal made from 100 parts of the original limonite ore are admixed with 135 parts of the same ore and 70 parts of lime, preferably in the form of briquettes; the three components being ground to 100 mesh. The briquettes are fed to a bath of 280 parts molten iron refined to the desired carbon content. The metal formed in the briquette internal reaction added to the iron produces 400 parts of steel containing 0.5 per cent chromium and 0.44 per cent nickel with less than 0.10 per cent carbon. The slag is lime silicate containing about 1.4 parts CaO to 1 SiO<sub>2</sub>. The ratio of slag to the steel produced is about 0.3:1. It is noted that it is not necessary to remove carbon from low chromium iron when a low chromium steel is produced. Carbon adjustments are readily made to give the desired carbon content in the steel.

If in the above embodiment a higher chromium steel is desired, then instead of removing the

silicon from the siliconized metal entirely with iron ore, I may add to the iron ore a desired ratio of calcium ferrichromite-chromate of any required high chromium content, as described in my accompanying application Serial No. 186,466. 5 An artificial chromite for this purpose is disclosed in my copending application Serial No. 165,417, filed September 23, 1937. The artificial chromite or calcium ferri-chromite-chromate may be made to great advantage by roasting high carbon ferro-chromium of any Cr/Fe ratio in finely divided admixture with lime and a little soda ash at about 1000° C. The roasted product is composed of CaO, Fe<sub>2</sub>O<sub>3</sub>, Cr<sub>2</sub>O<sub>3</sub> and CrO<sub>3</sub> in chemical combination, the lime being most advantageously in proportion to flux the silica formed in exothermic reduction of the chromium and iron oxides by silicon. It is noted that a greater content of silicon than 30 per cent may be put into the ferro-chrome silicon metal to supply a greater amount of heat to the steel furnace in the exothermic mixture. Instead of adding to this silicon content, it may be advantageous to use ferrosilicon or silicon in admixture with ferrochrome silicon and iron ore. 20

In the accompanying drawing, I have shown for purposes of illustration only, and not for purposes of limitation, a flow sheet illustrating several of the possible chromium recovery processes which may be carried out in employing the principles of the invention. Heavy lines have been employed to outline a complete process commencing with the treatment of ore containing chromium and iron and indicating the production ultimately of desirable chromium-bearing metal products. In dotted lines, there is indicated a modified process employing oxidized ferrochromium, and, in light lines, I have indicated the use of alloying elements such as nickel, molybdenum, manganese, vanadium and tungsten. 30

What I claim is:

1. As a composition useful in making alloy steels containing chromium, an intimate mixture of iron oxide, ferrochrome silicon low in carbon and containing sufficient silicon to reduce all the iron oxide to metal and lime sufficient to flux the silica formed in said reduction, said composition being capable of converting itself by internal exothermic reactions into a ferrous chromium alloy and a basic lime silicate slag. 45

2. A material for making chromium alloy steel composed of iron oxide, low carbon ferrochrome silicon containing silicon sufficient to reduce the iron oxide to metal and lime sufficient to flux the silica formed in said reduction to a basic silicate slag, all in finely divided admixture capable of converting itself by internal exothermic reaction into chromium alloy steel and lime silicate slag. 55

3. A material according to claim 2 in which the proportions of the three components in finely divided admixture are such as to form by exothermic reaction molten alloy steel and molten slag. 60

4. A silico-thermic material comprising a mixture of iron oxide, lime and siliconized ferro-chromium of controlled carbon content in finely divided condition and in proportions to form by internal exothermic reaction lime silicate slag having more than an equimolecular ratio of lime to silica and a chromium-iron metal of predetermined carbon and silicon contents. 65

5. A silico-thermic material comprising a mixture of iron oxide, lime, siliconized ferrochromium of controlled carbon content and a saline oxidant in finely divided condition and in proportions to form by internal exothermic reaction low-carbon

ferrous metal alloyed with chromium and lime silicate slag having more than an equimolecular ratio of lime to silica. 5

6. A silico-thermic material composed of iron oxide, nickel oxide, siliconized ferrochromium, a saline oxidant and lime in finely divided intimate admixture in relative proportions such as to form by internal exothermic reactions low silicon ferrous metal alloyed with chromium and with nickel and lime silicate slag having a CaO:SiO<sub>2</sub> molecular ratio greater than 1:1. 10

7. A process of making chromium alloy steel or iron from chromite ores which comprises reducing a chromite ore with carbon at a smelting temperature to high carbon ferrochromium with fluxing elimination of the ore gangue, siliconizing and removing carbon from said ferrochromium by smelting with silica and carbon, grinding said siliconized metal and mixing it with finely divided iron oxide and lime and igniting the mixture. 15

8. In utilizing natural ferrous chromite ores for making chromium alloy steels, a process which comprises reducing such an ore of any grade with carbon to high carbon ferrochromium, smelting said ferrochromium with silica and carbon to ferrochrome silicon high in silicon and low in carbon, admixing said ferrochrome silicon in finely divided form with finely divided lime and finely divided iron oxide in relative quantities such as to convert most of the silicon to calcium silicate and igniting said admixture to react exothermically and form the finished chromium alloy with calcium silicate slag. 20

9. In making chromium-iron alloys, a method of utilizing chromite ores which comprises making from chromite ore of any grade ferrochrome-silicon metal of high silicon content insuring a low carbon content, grinding said metal and mixing it with finely divided iron oxide and lime and igniting said mixture to form a low carbon chromium-iron metal by exothermic reaction. 30

10. In making chromium alloy steel or iron, a method of utilizing chromite ores which comprises making from chromite ore of any grade ferrochrome silicon metal of high silicon content insuring a low carbon content, grinding said metal and mixing it with finely divided iron oxide, a saline oxidant and lime in quantities sufficient to oxidize said silicon and igniting said mixture to form a chromium-iron metal by exothermic reaction. 45

11. A method of making low carbon chromium steel from low grade chromite ores of high iron content which comprises making from such an ore having a chromium-iron ratio less than 2:1 55 a ferrochrome-silicon metal of high silicon content insuring a low carbon content, grinding said metal and mixing it with finely divided iron oxide and lime and igniting said mixture to form a chromium-iron metal by exothermic reaction 60 with formation of a lime-silicate slag.

12. A silico-thermic material composed of ferro-chrome silicon metal having a Cr/Fe ratio less than 2:1, iron oxide and lime in an intimate mixture of particle sizes passing a screen of 100 65 meshes to the linear inch and capable of converting itself by internal exothermic reactions into chromium alloy steel and lime-silicate slag.

13. A method of making a silico-thermic material for use in producing chromium-iron alloys 70 which comprises, fine-grinding a ferrochrome silicon metal of high silicon and correspondingly low carbon content and intimately mixing the ground metal with finely ground iron oxide and lime in about the quantities required to oxidize the sili- 75

con of the metal with formation of a lime-silicate slag containing lime in at least an equimolecular ratio to the silica.

14. A material for use in making alloy steel

5 by exothermic action which comprises an intimate mixture of finely divided iron oxide, ferrochrome silicon and burned lime, the lime being in a ratio to the silicon of the ferrosilicon somewhat greater than 2 parts by weight of lime to 10 one part of silicon.

15. A silico-thermic material capable of converting itself by internal exothermic reaction into nickel-chromium alloy steel, said material being an intimate mixture of iron oxide, a ferrochrome silicon metal containing nickel and lime in proportions to oxidize the silicon to a lime-silicate slag having a CaO—SiO<sub>2</sub> molecular ratio above 1:1.

16. A method of producing a composition for 20 use in making alloy steels containing chromium which comprises grinding to a fineness at least sufficient to pass a screen of 100 meshes to the inch a mixture of iron oxide, ferrochrome silicon low in carbon and containing sufficient silicon to reduce all the iron oxide to metal and

lime sufficient to flux the silica formed in said reduction to a lime silicate slag containing lime in a ratio greater than one mol CaO to one mol SiO<sub>2</sub>.

17. As a composition useful for the production of chromium alloy steel, an intimate mixture consisting essentially of iron oxide, a saline oxidant, ferrochrome silicon containing silicon in amount sufficient to reduce the iron oxide to metal and to be oxidized by the saline oxidant and lime sufficient to flux the silica formed by oxidation of said silicon, said composition being capable of converting itself by internal exothermic reactions into a ferrous chromium alloy and a basic lime silicate slag.

18. A silico-thermic material comprising a mixture of oxidized ferrochromium, iron oxide, lime and ferrochrome silicon of controlled carbon content in finely divided condition and in proportion to form by internal exothermic reaction lime silicate slag having more than an equimolecular ratio of lime to silica and a chromium-iron metal of predetermined carbon and silicon contents.

MARVIN J. UDY. 25